

# United States Patent

[19]

Malm et al.

[11] 3,720,998

[45] March 20, 1973

[54] **METHOD OF MANUFACTURING  
COMMUTATOR SEGMENTS OF  
COMPOUND MATERIAL**

[75] Inventors: Assar Malm; Jan-Erik Fransson,  
both of Vasteras, Sweden

[73] Assignee: Allmanna Svenska Elektriska Ak-  
tiebolaget, Vasteras, Sweden

[22] Filed: May 6, 1971

[21] Appl. No.: 140,687

[52] U.S. Cl..... 29/597

[51] Int. Cl. .... H01r 43/00

[58] Field of Search ..... 29/597; 72/60; 310/233

[56] **References Cited**

## UNITED STATES PATENTS

1,898,696 2/1933 Sorensen ..... 29/597  
1,314,051 8/1919 Doman ..... 29/597  
3,478,421 11/1969 Preece ..... 29/597

3,620,059 11/1971 Nilsson ..... 72/60

## OTHER PUBLICATIONS

ASEA Inc. Bulletin; Pamphlet AQ 14-106E; covering  
"Production of Copper-Clad Aluminum a New QUIN-  
TIS Process"; September, 1970.

Primary Examiner—Richard J. Herbst  
Attorney—Jennings Bailey, Jr.

[57] **ABSTRACT**

Commutator segments are formed by hydrostatically extruding a billet having a core of aluminum or aluminum alloy and a tubular copper or copper alloy casting through a die of such shape that a thin strip is produced. This strip, either during extending or by rolling after extrusion, is given a shape which is thinner in the center than at the edges. The strip is cut longitudinally along its central axis and cut to suitable lengths.

**4 Claims, 4 Drawing Figures**



PATENTED MAR 20 1973

3,720,998

Fig. 1



Fig. 2



Fig. 3



Fig. 4



INVENTOR.

ASSAR MALM  
BY JAN-ERIK FRANSSON  
Jennings Barley, Jr.

## METHOD OF MANUFACTURING COMMUTATOR SEGMENTS OF COMPOUND MATERIAL

### BACKGROUND OF THE INVENTION

#### 1. Field of the Invention

The present invention relates to a method of manufacturing commutator segments of compound material having a core of aluminum and a casing of copper on at least one, but usually three, of the side surfaces of the segment.

#### 2. The Prior Art

Usually commutators are built up of segments having substantially wedge-shaped cross-section and consisting of copper or a copper alloy with copper as the main constituent. Experiments have also been carried out to manufacture commutator segments having substantially rectangular or slightly wedge-shaped frames of a material, normally steel or aluminum, and contact rails of pure copper or a copper alloy applied on one of the narrow sides of the frame. Because of the weight and the forces arising during rotation, which among other things give rise to bending and skewing stresses in the segments and tensile stresses in so-called pressure rings holding together a collector packet, it is desirable to use a light material for the frame. Because of its low weight, aluminum is a suitable material. However, it is extremely difficult to join copper and aluminum satisfactorily. At temperatures above about 450° copper and aluminum form brittle alloys. When copper and aluminum rails are joined by means of welding or soldering, a brittle layer is formed in the contact region between the materials, which reduces the strength. Copper and aluminum have different coefficients of thermal expansion so that shearing stresses arise in the joint upon temperature fluctuations. The risk of breaking of welded or soldered joints is thus considerable.

It has also been proposed to manufacture commutator segments by electrolytically providing one surface on the frame of the commutator segment with a contact surface of copper. However, copper which is applied electrolytically does not have suitable structure and the required strength for commutator purposes. The bond between copper and aluminum is normally also unsatisfactory with electrolytic application. The savings in the quantity of copper have so far not usually outweighed the costs of producing bimetallic commutator segments with low copper content and the inconvenience and risks of using commutators constructed of such segments.

#### Summary of the Invention

The method according to the invention makes it possible to produce a bimetallic commutator segment having a core consisting essentially of aluminum and a contact surface consisting essentially of copper which, from the technical point of view, provides a satisfactory replacement for commutator segments of solid copper. Furthermore, in many cases the decreased weight is a considerable advantage. The weight can be reduced by 40–60 percent depending on the desired wear depth on the segments. The lower weight of the segments causes a reduction in centrifugal forces which, in turn, causes reduced bending and skewing stresses in the segments themselves and less strain on the pressure rings which hold together the stack of segments forming the commutator. The reduction in stresses permits reduced

height of the segment, which is also a saving in material. Usually the outer diameter remains unaltered. It is thus possible to arrange larger cooling channels inside the commutator. A smaller and lighter commutator 5 also involves a lower moment of inertia which, particularly in some cases, may be of great value.

The satisfactory features of the commutator segments are due partly to the direct metallic bond between the copper in the casing and the aluminum in 10 the core or frame and partly to the fact that the frame is surrounded by copper on at least three sides. If the core is surrounded on all sides by copper and the quantity of copper is symmetrically placed, no deformation is caused by temperature fluctuations. Even with three-sided, U-shaped copper casings, the copper in the legs of the U contributes to limiting the deformation caused by temperature fluctuations.

In the method according to the invention, the metallic bond between aluminum and copper is obtained by 20 means of isostatic extrusion of a billet having a core of aluminum or an aluminum alloy and a casing of copper or a copper alloy surrounding the core, according to the methods described in Swedish Pat. Nos. 318,540 and No. 327,180, so that a section is obtained which has a large ratio between width and height. After the extrusion, the section is split into two similar sections which are then surrounded by copper on three sides. During the extrusion a rectangular section may be 25 produced, which is rolled to double wedge-shaped cross-section, from which segments having the desired wedge shape are obtained by splitting the section and cutting it into suitable lengths. It is also possible during the extrusion to give the section the desired cross-section directly, thus eliminating one operation.

The method offers a wide selection of material. For instance, a high-strength aluminum alloy may be used in the core and a copper alloy suitable from the point of view of wear for the casing. With previous methods of 30 combining these materials, attempts to produce a compound product have been unsuccessful. The casing may consist of a copper alloy containing at least 99 percent copper and silver (Cu + Ag) or some other alloy suitable for commutator purposes. The core may consist of 35 pure aluminum, but a high-strength alloy containing 3.5–5.0% Cu, max. 1.0% Si, max. 1.0% Fe, 0.5–1.0% Mn, max. 1.0% Zn, 0.4–1.8% Mg, 1.0–3.0% Pb+Sn+Bi+Cd+Sb, max. 0.2 percent grain refinement additives and the remainder Al is particularly 40 suitable.

It is possible to produce segments having a cross-section consisting of 10–40 percent copper.

The difference in price between copper and aluminum is considerable. The reduction of the quantity 45 of copper therefore involves a considerable decrease in costs. The raw material cost of a segment may drop by up to 70 percent if there is only a small copper content. For a commutator segment having a height of 50 mm and a thickness of 10 mm at the bottom of the U-shaped casing, the costs may be reduced by 30–40 percent.

#### Brief Description of the Drawings

The invention will be described further with reference to the accompanying drawings.

FIG. 1 shows a side view and FIG. 2 a section of a commutator segment produced by the method according to the invention.

FIGS. 3 and 4 show sections of compound material produced by extrusion, which form an intermediate product in the production of segments having the cross section shown in FIG. 2.

#### Description of the Preferred Embodiments

In the drawings 1 designates a commutator segment which is provided at the ends with triangular cuts 2 to receive pressure rings which hold together the segments in a commutator. The segment comprises a core 3 of an aluminum alloy and a U-shaped copper casing 4 which surrounds three sides of the core 3. The thickness of the casing varies. The casing is considerably thinner on the long sides 5 of the core than on its short side 6 which forms the contact surface in a commutator. With a segment height of 50 mm it is possible to obtain a thickness of 10 mm or more on the short side 6 of the segment. The segment is slightly wedge shaped and the wedge incline is chosen so that the planes of the side surfaces meet each other at the center line of a finished commutator. To manufacture the segment, a compound billet is used to start with which consists of an aluminum core and a tubular casing, which are extruded directly to a section according to FIG. 3 having a double wedge-shaped cross-section with the desired cross-section, or to a section according to FIG. 4 which, after the extrusion, is rolled to a double wedge-shaped cross-section according to FIG. 3. The section according to FIG. 3 is then split lengthwise

transversely of its width to produce the segment according to FIG. 2.

We claim:

1. Method of manufacturing commutator segments with a core consisting essentially of aluminum and a casing consisting essentially of copper, which comprises hydrostatically extruding a billet of compound material including a core consisting essentially of aluminum and a casing consisting essentially of copper into a strip of relatively thin cross-section compared to its width, whereby to bond the casing and core together, and splitting the strip longitudinally transversely of its width.
- 15 2. Method according to claim 1, in which the step of extruding includes making the strip thinner along its longitudinal center line than at its edges.
- 20 3. Method according to claim 1, in which the step of extruding includes making the strip of substantially rectangular cross-section, the step of forming the extruded billet to a double wedge-shaped cross-section before splitting the strip, said cross-section being thinner along the longitudinal center line of the strip than at its edges.
- 25 4. Method according to claim 1, in which the step of extruding includes making the material of the casing substantially thicker on the edges of the strip than on its flat sides.

\* \* \* \* \*

30

35

40

45

50

55

60

65

UNITED STATES PATENT OFFICE  
CERTIFICATE OF CORRECTION

Patent No. 3720998

Dated March 20, 1973

Inventor(s) Assar Malm and Jan-Erik Fransson

It is certified that error appears in the above-identified patent  
and that said Letters Patent are hereby corrected as shown below:

After the heading, insert:

Claims priority, Application Sweden,  
May 6, 1970, 6273/70.

Signed and sealed this 10th day of July 1973.

(SEAL)

Attest:

EDWARD M. FLETCHER, JR.  
Attesting Officer

Rene Tegtmeier  
Acting Commissioner of Patents